

# UNITED STATES PATENT OFFICE.

ROBERT DENIS LANCE, OF LIVRY, FRANCE, ASSIGNOR OF ONE-HALF TO CÉCIL SHRAGER, OF LONDON, ENGLAND.

## ARTIFICIAL SILK.

1,398,525.

Specification of Letters Patent. Patented Nov. 29, 1921.

No Drawing.

Application filed April 1, 1913. Serial No. 758,245.

(GRANTED UNDER THE PROVISIONS OF THE ACT OF MARCH 3, 1921, 41 STAT. L., 1313.)

To all whom it may concern:

Be it known that I, ROBERT DENIS LANCE, a citizen of the French Republic, and a resident of Livry, Seine-et-Oise, France, 18 Rue 5 Saint-Claude, gentleman, have invented certain new and useful Improvements in and Relating to Artificial Silk, (for which I have filed applications in France April 9, 1912; in Germany April 13, 1912,) of which the following is a complete specification.

It is known that viscose or nitro cellulose silks present the defect of offering less resistance in a dry state to various influences and particularly to water than natural silk.

15 This invention has for its object artificial viscose and nitro cellulose silks of great strength and from which fabrics that can even be washed in boiling water can be formed.

20 The process of making the silk which forms the object of the invention consists mainly in adding to solutions of viscose or nitro-cellulose metallic resinate, in particular resinate of zinc or of magnesium or a 25 mixture of the two presenting a very high fusion point and for obtaining a pliable final product the percentage of resinate in the solution should not preferably exceed 20%. This proportion of resinate can, 30 however, be exceeded if highly oxidized siccative oils, stearin, elaidin or a mixture of these bodies be added to the mixtures of viscose or cellulose and resinate. If an excess of metallic resinate be employed a hard 35 product analogous to celluloid is obtained. It is known to mix nitro cellulose moistened with a solution of sulfuric acid with siccative oils previously treated with sulfur chlorid. It has also been proposed to add 40 to the solution a solution of caoutchouc and to vulcanize the mixture with sulfur chlorid or to coat the thread obtained by means of this mixture with albumin which is coagulated by the sulfur chlorid. As additional body caoutchouc mixed with zinc chlorid has also been used, as have metallic 45 resinate treated with saltpeter. For obtaining plastic masses of the celluloid type resinous alkaline soaps with a soda or a 50 potash base have also been mixed with nitro cellulose.

All these ingredients, however, do not fur-

nish a utilizable silk, strong when dry and when in a humid state. In accordance with the present invention such a silk is obtained 55 by adding metallic resinate to cellulose esters such as a solution of viscose or of nitro cellulose and then spinning the mixture. From this point of view the novel process is also differentiated from the known process 60 consisting in impregnating threads and fabrics for example with resinate of aluminum, a process by which the threads only receive an excessively thin layer of resinate while when the resinate are incorporated 65 in the solution, the thread manufactured is completely impregnated with these resinate and consequently forms a body which is almost completely impermeable.

It is known that the fusion point of resins, 70 balsams and gum-resins is considerably raised by the addition of zinc oxid or magnesium oxid.

For example, the addition of 4% of zinc oxid to a colophony brings its fusion point 75 from 70° to 125°; 8% from 70° to 170° a temperature which enables it to withstand a heat of 100° without softening in a manner harmful to the silk.

In a cold state, the resinate prevent the 80 silk from being penetrated by water and enable it to retain great strength. They render it proof against soap washing or washing with alkaline carbonates.

These metallic resinate can be added to 85 solutions of viscose or of nitro cellulose in any proportions; as however these resinate are hardening agents and consequently present the property of destroying the elasticity of manufactured products, they must not be 90 employed in proportions which, generally speaking, exceed 20%, if it be desired to preserve adequate pliability in the final product.

If it be desired to use higher proportions 95 and still obtain pliable products, it is necessary to add to the mixtures either siccative oils that have already been highly oxidized, or, and preferably, stearin or better still elaidin or a mixture of these three bodies. 100

In increasing the proportion of resinate, especially if aluminum resinate be employed without employing in conjunction therewith the products previously referred to, bodies

of the nature of celluloid are manufactured and these bodies can replace celluloid in many of its applications.

The resinates are obtained in the following manner: The resins, the balsams or the gum-resins, according to circumstances, or a mixture of these products is dissolved in carbon disulfid or ether, according as it is desired to incorporate the resinate with viscose or with nitro cellulose, oxids or hydroxids of zinc or of magnesia or a mixture of the two substances are then added in the proper proportion for the product to be obtained, the whole being then agitated until solution takes place.

The carbon disulfid containing the resinate or resinates serves, in the ordinary way, for dissolving the alkali-cellulose; similarly the resinated ether mixed with alcohol, benzoin or acetone serves to dissolve the nitro cellulose.

The addition to the resinates of zinc or of magnesium, or to the mixture of the two with resinate of aluminum or of tungsten even in small proportions (0.5%) serves to diminish the combustibility of the products obtained by means of nitro cellulose and consequently of avoiding or reducing the denitration.

The spinning of solutions of resinated viscose takes place in the same baths as ordinary viscose. Resinated collodion is spun in the air like ordinary collodion. For the preparation of the viscose with a view to this manufacture, it is advantageous for obtaining alkali-cellulose to substitute an alcoholic soda lye for an aqueous lye. The reaction takes place in the same manner and

more speedily; furthermore, the alkali-cellulose thus obtained dissolves more readily in the resinated carbon disulfid.

Apart from the advantages referred to above which are inherent in the product obtained by this novel process the employment of metallic resinates, particularly in the case of nitro cellulose silk, presents the advantage that the nitro cellulose is highly diluted by the relatively large quantity of resinates and that its combustibility is greatly diminished by reason of the small combustibility of the metallic resinates. As, on the other hand, the thread loses some of its tenacity owing to the denitration, the silk that is not denitrated or only incompletely denitrated in accordance with the novel process, notwithstanding the small proportion of nitro cellulose that it contains, presents greater strength because the nitro cellulose of which it is composed is firmer.

What I claim is:

1. An artificial silk comprising a cellulose ester having a metallic resinate with a high fusion point, said resinate not exceeding 20%.
2. An artificial silk comprising a cellulose ester, a metallic resinate having a high fusion point, and a highly oxidized siccative oil.

In testimony whereof I have hereunto placed my hand at Paris, France, this eleventh day of March 1913.

ROBERT DENIS LANCE.

In the presence of two witnesses:

Louis Coquillat,  
Lucien Menninger.